

# United States Patent [19]

Matsumoto et al.

[11] 3,871,884

[45] Mar. 18, 1975

[54] **PHOTOCONDUCTIVE COMPLEX WITH HYDROXY-NITROBENZOIC ACIDS AND TRIARYLMETHANE DYES**

[75] Inventors: **Shoichi Matsumoto, Kazuhiko Kurematsu**, both of Yokohama, Japan

[73] Assignee: **Tokyo Shibaura Electric Co., Ltd.**, Kawasaki-shi, Japan

[22] Filed: **Dec. 14, 1971**

[21] Appl. No.: **207,981**

[30] **Foreign Application Priority Data**

Dec. 16, 1970 Japan..... 45-11880

[52] U.S. Cl..... **96/1.6, 96/1.5**

[51] Int. Cl..... **G03g 5/06**

[58] **Field of Search**..... 96/1 R, 1 PC, 1.5, 1.6

[56] **References Cited**

UNITED STATES PATENTS

3,037,861 6/1962 Hoegl et al. .... 96/1.5

|           |         |                       |        |
|-----------|---------|-----------------------|--------|
| 3,159,483 | 12/1964 | Behmenburg et al..... | 96/1.5 |
| 3,162,532 | 12/1964 | Hoegl et al. ....     | 96/1.5 |
| 3,287,120 | 11/1966 | Hoegl.....            | 96/1.5 |
| 3,421,891 | 1/1969  | Inami et al. ....     | 96/1.6 |

*Primary Examiner*—Roland E. Martin, Jr.

[57] **ABSTRACT**

Photoconductive materials for electrophotography have been formed by blending a molecular compound produced by a charge transfer reaction of poly-N-vinylcarbazole and tetrachloro-p-benzoquinone, with at least one compound selected from the group consisting of 2-hydroxy-3,5-dinitrobenzoic acid, 2-hydroxy-3-nitrobenzoic acid and 2-hydroxy-5-nitrobenzoic acid, and with at least one triarylmethane dyestuff. These photoconductive materials for electrophotography are not only characterized by high sensitivity and excellent image quality, but they also can be easily cast into films and possess good transparency.

**5 Claims, No Drawings**

## PHOTOCONDUCTIVE COMPLEX WITH HYDROXY-NITROBENZOIC ACIDS AND TRIARYLMETHANE DYES

### BACKGROUND OF THE INVENTION

#### 1. Field of the Invention

This invention relates to a photoconductive material for electrophotography having high sensitivity, excellent image quality, and good transparency, and which has good film castability.

#### 2. Description of the Prior Art

Inorganic materials, such as selenium or zinc oxide, and organic materials, such as poly-N-vinyl carbazole systems or polyacetylnaphthylene systems, have been used as photoconductive materials by the prior art. The organic photoconductive materials in particular have been considered to be especially attractive industrially, since they can be easily cast into films, they possess high flexibility which renders them easily handleable, and they can be formed at relatively low costs. Nevertheless, the conventional organic materials used for this purpose have demonstrated several undesirable defects which have prevented the attainment of higher image quality, and higher photosensitivity. For instance, although poly-N-vinyl carbazole has good spectral sensitivity in the ultraviolet region, its degree of sensitivity is so low that it has insufficient electrophotographic sensitivity under incandescent light exposure. Attempts have been made to improve this sensitivity by blending a small amount of tetrachloro-p-benzoquinone as a sensitizer, with the poly-N-vinyl carbazole, in order to shift the spectral sensitivity to the visible regions and at the same time to intensify the photosensitivity. However, these attempts have not been entirely successful, since they have resulted in compositions possessing rather poor resolution, and which are characterized by non-uniformity of image, strong edge effects, and staining of the non-imaged parts. In another piecemeal attempt to eliminate these defects, several dye sensitizers were further blended with the poly-N-vinylcarbazole/tetrachloro-p-benzoquinone mixture, but such attempts have been met with only limited success. Thus, it is difficult to satisfactorily use these organic photoconductive materials for electrophotography purposes.

A need exists, therefore, for an electrophotography photoconductive material which is not only characterized by high sensitivity and excellent image quality, but also can be easily cast into films of good transparency.

### SUMMARY OF THE INVENTION

Accordingly, it is one object of this invention to provide an organic photoconductive material for electrophotography which is not only characterized by high sensitivity and excellent image quality, but also by easy film castability for films and good transparency.

This and other objects have now herein been attained by providing a photoconductive material for electrophotography formed by blending a molecular compound produced by a charge transfer reaction of poly-N-vinyl carbazole and tetrachloro-p-benzoquinone, with at least one compound selected from the group consisting of 2-hydroxy-3,5-dinitrobenzoic acid, 2-hydroxy-3-nitrobenzoic acid and 2-hydroxy-5-nitrobenzoic acid, and with at least one triarylmethane dyestuff.

Tetrachloro-p-benzoquinone is not only a sensitizer for poly-N-vinylcarbazole, but since they effectively overlap each other in their molecular orbital electronic states, their reaction product by charge transfer reaction possesses excellent photoconductive properties which is highly suitable for electrophotography.

It has now been found that when this molecular compound is blended with a derivative of benzoic acid and a dye sensitizer, a photoconductive material characterized by excellent electrophotography properties is obtained.

### DETAILED DESCRIPTION OF THE INVENTION

The above-mentioned molecular compound, which is the main component of the photoconductive materials of this invention, can be obtained quite easily, as follows:

A solution of poly-N-vinyl carbazole and a solution of tetrachloro-p-benzoquinone is prepared. Both solutions are heated slightly and the poly-N-vinyl carbazole solution is added to the tetrachloro-p-benzoquinone solution while stirring vigorously. Stirring is continued for several hours and the combined solutions are concentrated slowly and left for several hours at room temperature. A non-soluble solvent, such as methylalcohol, is then added slowly to the mixed solution, while stirring, until a deep blue violet-colored deposit is produced as a fine suspension in the solution. The separated, refined and dried deposit will be the charge transfer reaction product of poly-N-vinylcarbazole and tetrachloro-p-benzoquinone. The reaction may conveniently be carried out at temperatures of about 50°C. and in such solvents as chloroform.

35 A benzoic acid derivative compound, such as 2-hydroxy-3,5-dinitrobenzoic acid, 2-hydroxy-3-nitrobenzoic acid or 2-hydroxy-5-nitrobenzoic acid, is then mixed and blended with the molecular charge transfer reaction product in a ratio of 0.5-10 parts by weight of the benzoic acid derivative per 100 parts of charge transfer reaction product.

30 0.05-2 parts by weight of a triarylmethane dyestuff per 100 parts by weight of the charge transfer reaction product is then added to the blend.

45 Suitable triarylmethane dyestuffs which can be used for this purpose include crystal violet, Brilliant-green, Victoria blue, Methyl violet, Malachite green, Acid violet 6B, etc.

The photoconductive material of this invention can be further blended with p-ter-phenyl, diphenyl, diphenylchloride, dibutylphthalate, dimethylglycolphthalate, triphenylphosphate, methylnaphthalene or diocetylphthalate, etc. as a plasticizer to improve its film-forming capability.

55 The charge transfer reaction product, however, is a high molecular weight compound, which possesses good film formability and good flexibility even without the optional plasticizer, and it possesses good transparency and high sensitivity throughout the visible region. It is highly photoconductive itself, without any other additive, but when it is blended with one of the above-mentioned benzoic acid derivatives, and at least one triarylmethane dyestuff, it becomes even more highly sensitive. Surprisingly, when this product is blended with only the benzoic acid derivative or with only the triarylmethane dyestuff separately, the degree of sensitivity and image quality tends to be lower, rather than improved.

The photoconductive film produced by the photoconductive material of this invention can be formed with good homogeneity and is characterized by good image reproducibility when exposed through any colored original incandescent light or other visible rays, and can form an image of good resolution and high uniformity. Moreover, when the substratum is moderately transparent, the image formed can be used as a so-called "secondary master," as a substitute for a negative or a semitransparent master, i.e., a diazo master or a copy master.

The reason why the photoconductive material of this invention has such good photographic characteristics is not fully understood, but seems to be explainable as follows: The charge transfer reaction product is formed from poly-N-vinylcarbazole and the tetrachloro-p-benzoquinone, which effectively overlap each other in molecular orbital electronic states. This is believed to have some effect in increasing the sensitivity. When this product is combined with the benzoic acid derivative and the triarylmethane dyestuff, the sensitivity becomes even greater. Moreover, the charge transfer reaction product which forms the matrix of the system is a high molecular weight material which possesses good miscibility in the blend and permits the formation of a smooth and homogeneous photoconductive film.

Having now generally described the invention, a further understanding can be attained by reference to certain specific Examples which are provided herein for purposes of illustration only and are not intended to be limiting unless otherwise so specified.

#### EXAMPLE

A chloroform solution of poly-N-vinylcarbazole (hereinafter referred to as solution A) was prepared by dissolving 4.0 g. of poly-N-vinylcarbazole in 1.4 l. of chloroform.

Another chloroform solution of tetrachloro-p-benzoquinone solution (hereinafter referred to as solution B) was prepared by dissolving 4.9 g. of tetrachloro-p-benzoquinone in 1.0 l. of chloroform. Solution A was heated to a temperature of 50°C. and was added dropwise into solution B which was also heated to a temperature of 50°C. The mixing was accompanied by vigorous stirring. After the mixing of solutions A and B, stirring was continued for 3 hours and the temperature was maintained at 50°C. The mixed solution was then concentrated slowly to a volume of 1 liter, and was left for 24 hours at room temperature.

160 ml. of methyl alcohol was then dripped into the concentrated solution, while stirring, and a deep blue

violet-colored deposit was produced as a fine suspension in the solution. This deposit was separated from the solution, refined and dried. This was identified as a molecular compound produced by a charge transfer reaction of poly-N-vinylcarbazole and tetrachloro-p-benzoquinone.

As shown in Table I, the six photoconductive materials for electrophotography were prepared by selecting and blending the above-mentioned poly-N-vinylcarbazole-tetrachloro-p-benzoquinone molecular compound (hereinafter referred to as PVCA.CHLO molecular compound), one compound selected from the group consisting of 2-hydroxy-3,5-dinitrobenzoic acid, 2-hydroxy-3-nitrobenzoic acid and 2-hydroxy-5-nitrobenzoic acid, and a triaryl methane dyestuff.

0.5 g. of photoconductive material for electrophotography was prepared and dissolved in 9 ml. of a chloroform-acetone mixed solvent (5 : 1). The solution obtained was added dropwise onto the surface of an aluminum plate (1 mm. in thickness), dried and formed into a photoconductive film (10 $\mu$  in thickness). Six photosensitive plates for electrophotography were prepared, and these plates were given a positive electric charge by ordinary corona-discharge methods from a 5 kV. source. The plates were then exposed with incandescent light through an original master by means of photographic enlarger, and were developed by cascading the toner. The optimum exposure of the photosensitive plates for electrophotography obtained as above described, was measured and is shown in Table I.

The "optimum exposure" described here, means the so-called optimum exposure required to obtain a faithful duplication of the original master of good resolution or good contrast, uniform image, stainlessness of the non-imaged portions and to produce a copy of good image quality without edge effects.

As controls for photosensitive plates prepared by blending of (1) PVCA.CHLO molecular compound, and (2) at least one compound selected from the group consisting of 2-hydroxy-3,5-dinitrobenzoic acid, 2-hydroxy-3-nitrobenzoic acid and 2-hydroxy-5-nitrobenzoic acid, was observed and measured experimentally and was measured for optimum exposure. The optimum exposure of materials prepared by blending (1) PVCA.CHLO molecular compound, and (3) a triarylmethane dyestuff, was observed and measured experimentally. The optimum exposures were both 90-160 lux.sec. which was inferior or only as good as the optimum exposure of photosensitive plates pre-

TABLE I

| Component                         | SAMPLE |     |     |     |     |     |
|-----------------------------------|--------|-----|-----|-----|-----|-----|
|                                   | 1      | 2   | 3   | 4   | 5   | 6   |
| (parts by wt.)                    |        |     |     |     |     |     |
| PVCA.CHLO molecular compound      | 100    | 100 | 100 | 100 | 100 | 100 |
| 2-hydroxy-3,5-dinitrobenzoic acid | 4.0    | 6.0 | —   | —   | —   | —   |
| 2-hydroxy-3-nitrobenzoic acid     | —      | —   | 2.0 | 7.5 | —   | 5.0 |
| 2-hydroxy-5-nitrobenzoic acid     | —      | —   | —   | —   | 1.0 | —   |
| Crystal violet                    | 0.5    | —   | —   | —   | —   | 0.2 |
| Brilliant green                   | —      | 1.0 | —   | 1.4 | —   | 0.5 |
| Victoria blue                     | —      | —   | 0.3 | —   | 0.2 | —   |
| Optimum exposure (lux.sec.)       | 21     | 17  | 24  | 28  | 31  | 25  |

pared by (1) PVCA.CHLO molecular compound alone, which was about 100 lux.sec.

As another control, the optimum exposure of photo-sensitive plates prepared by blending poly-N-vinylcarbazole, and tetrachloro-p-benzoquinone, instead of (1) PVCA.CHLO molecular compound which was a main component of photoconductive material for electrophotography in each sample, was observed and measured experimentally, and found to be 700-1,000 lux.sec., respectively. The duplicated copy prepared was not only inferior in resolution and contrast, but had poor image uniformity and was highly stained in the non-imaged portion. Moreover, it was inferior in edge effect and image quality.

The photoconductive material of this invention is also rather superior to zinc oxide systems (ZnO) in photosensitivity, and forms a better image than either selenium and zinc oxide (ZnO) systems, as photoconductive film.

Having now fully described the invention, it will be apparent to one of ordinary skill in the art that many changes and modifications can be made hereto without departing from the spirit or scope of the invention. Accordingly,

What is claimed as new and desired to be secured by letters patent is:

1. A photoconductive material for electrophotog-

raphy comprising a blend of

a. a molecular charge transfer reaction product of poly-N-vinylcarbazole and tetrachloro-p-benzoquinone,

5 b. at least one benzoic acid derivative selected from the group consisting of 2-hydroxy-3,5-dinitrobenzoic acid, 2-hydroxy-3-nitrobenzoic acid and 2-hydroxy-5-nitrobenzoic acid, and

c. at least one triaryl methane dyestuff.

10 2. The photoconductive material of claim 1, wherein the ratio of the benzoic acid derivative to said charge transfer reaction product is 0.5 to 10 parts/100.

15 3. The photoconductive material of claim 1, wherein the triaryl methane dyestuff is selected from the group consisting of Crystal violet, Brilliant-green, Victoria blue, Methyl-violet, Malachite-green and Acid-violet 6B.

20 4. The photoconductive material of claim 1 which further contains a plasticizer selected from the group consisting of p-ter-phenyl, diphenyl, diphenylchloride, dibutylphthalate, dimethylglycolphthalate, triphenyl-phosphate, methylnaphthalene and dioctylphthalate.

25 5. The photoconductive material of claim 1 which contains 0.05-2 parts by weight of a triaryl methane dyestuff per 100 parts by weight of said charge transfer reaction product.

\* \* \* \* \*

30

35

40

45

50

55

60

65